

# UNITED STATES PATENT OFFICE.

GEORGE S. PAGE, OF STANLEY, NEW JERSEY, ASSIGNOR OF THREE-FOURTHS  
TO CHARLES E. BOOTH, OF NEW YORK, N. Y.

## MANUFACTURE OF PAPER FOR PACKING AND OTHER PURPOSES.

SPECIFICATION forming part of Letters Patent No. 242,840, dated June 14, 1881.

Application filed December 16, 1880. (No specimens.)

*To all whom it may concern:*

Be it known that I, GEORGE SHEPARD PAGE, a citizen of the United States, and a resident of Stanley, in the county of Morris and State of New Jersey, have invented certain new and useful Improvements in the Manufacture of Paper for Packing and other Purposes, of which the following is a full, clear, and exact description.

- 10 The object of my invention is to produce a fabric useful in the preservation of fruits, vegetables, meats, dairy products, &c., not only from decay, but from becoming wasted or insipid, without imparting to the same any obnoxious odor, or unfit it for culinary or edible purposes; and to this end my invention consists in saturating the paper with a composition of salicylic acid, resin, paraffine, crude turpentine, and pine-tar.
- 15 The solution or composition in which the paper or other material is saturated is composed of salicylic acid, ten (10) per cent.; resin, fifty (50) per cent.; paraffine, ten (10) per cent.; crude turpentine, fifteen (15) per cent.; pine-25 tar, fifteen (15) per cent. Steam or other heat is used as a reducing agent to form a chemical combination of all the elements. The paper is then passed through this compound, so as to thoroughly saturate the same, and is then freed 30 from any surplus of the saturating material by means of scrapers or pressure-rolls, and then passed in contact with heated surfaces or exposed to heated air-blasts, whereby the paper is rendered dry and cleanly. Any suitable or 35 proper machine may be used for the saturation and drying.

For some purposes it may be necessary to

substitute resin for the crude turpentine and pine-tar, and also to increase the percentage of paraffine and salicylic acid to some extent, 40 without departing from the spirit of my invention.

In some instances, where the odor is not injurious or objectionable, I may substitute for the salicylic acid naphthaline, or the naphthaline may be used in connection with the salicylic acid.

I do not limit myself to paper thus treated, for it is obvious that felted or woven fabrics could be saturated and used to advantage in 50 the same manner as the paper, and that woollen fabrics, furs, feathers, and like articles are preserved from the ravages of insects, and that metal surfaces are protected from rust and tarnish by being wrapped in the material or fabric prepared as above described.

Having thus described my invention, what I claim, and desire to secure by Letters Patent, is—

1. The compound herein described for saturating or coating paper, felt, woven fabric, or similar material, the same consisting of salicylic acid, resin, paraffine, crude turpentine, and pine-tar, as set forth.
2. As a new article of manufacture, paper or 65 similar fibrous or textile material saturated with the compound herein described, and treated in the manner set forth, for the purposes herein stated.

GEORGE SHEPARD PAGE.

Witnesses:

GEO. W. PEARSON,  
CHAS. E. BOOTH.